

July 25, 1972

H. B. BOMBERGER, JR., ET AL  
METHOD OF IMPROVING MACROSTRUCTURE  
OF TITANIUM-BASE ALLOY PRODUCTS  
Filed May 5, 1970

3,679,403



FIG. 1.



FIG. 2.

INVENTOR  
HOWARD B. BOMBERGER, JR.  
STANLEY R. SEAGLE  
By *Walter P. Wood*

Attorney

3,679,403

**METHOD OF IMPROVING MACROSTRUCTURE OF TITANIUM-BASE ALLOY PRODUCTS**

Howard B. Bomberger, Jr., Canfield, and Stanley R. Seagle, Warren, Ohio, assignors to RMI Company, Niles, Ohio

Continuation-in-part of application Ser. No. 749,269, Aug. 1, 1968. This application May 5, 1970, Ser. No. 34,674

Int. Cl. C22c 15/00

U.S. Cl. 75—175.5

9 Claims

**ABSTRACT OF THE DISCLOSURE**

A method of improving the macrostructure of titanium-base alloy products by adding to the alloy about 0.03 to 0.40 percent yttrium, which may be either the metal itself or a compound thereof. Addition of yttrium achieves a fine grain structure and avoids spangled surfaces on macroetched sections of the product, but usually lowers both the yield strength and ultimate tensile strength of the product. Invention compensates for this latter effect by adjusting the content of strengthening agents, preferably oxygen or nitrogen.

This application is a continuation-in-part of our earlier co-pending application, Ser. No. 749,269, filed Aug. 1, 1968, now abandoned.

This invention relates to a method of improving the macrostructure of titanium-base alloys and to the resulting product.

Coarse grain structures or a spangled surface condition interfere with sonic inspection of titanium-base alloy products. Either condition produces back-scatter or "noise" and thus makes the test less sensitive and may mask a defect. Also, coarse grain structures in welds and wrought products usually lead to poor mechanical properties, such as lower fatigue resistance and poorer workability. Fine grain structures can be developed in titanium-base alloys with sufficient mechanical working. Hence the problem of grain size is less acute in sheets or small size forgings, etc. Heavy sections and welds are not readily worked to the extent needed to develop fine grain structures. For example, the work performed in reducing a 30-inch diameter ingot of a titanium-base alloy to a 20-inch diameter billet is not sufficient for this purpose, and the billet usually is coarse-grained. Even though a product may be worked sufficiently to achieve a fine grain structure, macroetched sections of the product may have spangled surfaces which similarly hamper sonic inspection.

An object of the present invention is to provide a method of improving the macrostructure of titanium-base alloy products through yttrium additions without adversely affecting other properties.

A more specific object is to provide a method of improving the macrostructure of titanium-base alloy products in which we add yttrium to the alloy, but compensate for the adverse effect on tensile properties by increasing the content of strengthening agents, preferably oxygen and/or nitrogen.

A further object is to provide an improved titanium-base alloy product which results from practicing our method.

Our method is applicable to alloys which contain a minimum of about 70 percent by weight titanium. Most alloys for which our method is useful have a titanium content no greater than about 95 percent by weight, and our preferred range is about 70 to 95 percent titanium. Nevertheless our method may be useful for some alloys which have a titanium content as high as about 97 per-

cent by weight. The remainder of the alloy may consist of any combination of the usual alloying elements for titanium, including aluminum, tin, vanadium, zirconium, chromium, molybdenum, iron, oxygen, nitrogen and others. Our method is applicable to alloys which contain alpha and/or beta phases. Surprisingly it is not applicable to unalloyed titanium nor to alloys which contain less than about 3 percent by weight of alloying elements.

According to our method, we incorporate in the alloy about 0.03 to 0.40 percent by weight yttrium. Since yttrium is costly, we prefer to add it in the minimum quantity to achieve the desired improvement in macrostructure of the alloy. Additions of yttrium to produce a content in excess of our upper limit tend to make alloys more difficult to work, even though they may achieve the desired improvement in macrostructure. We may add yttrium to the alloy either in the form of the metal itself or a compound, such as the oxide  $Y_2O_3$ , provided the other elements in the compound have no adverse effect on the final alloy or are within allowable limits. We prefer to use a compound for reasons that compounds are less costly, and other elements of the compound may supply a strengthening agent, as hereinafter described. In adding yttrium to an alloy, we may follow the usual technique of combining yttrium metal or a yttrium compound with sponge titanium and the other alloying elements in a consumable electrode, and melting the electrode with an electric arc to form an ingot. Yttrium has little solubility in titanium, but tends to form a fine refractory oxide precipitate with a melting point above 4300° F., which is substantially higher than the melting point of titanium.

Table 1, which follows, demonstrates the benefits we have obtained in controlling the grain size of various titanium-base alloys by adding yttrium.

TABLE 1

|    | Composition, wt. percent:                        | Grain size <sup>1</sup> |                        |
|----|--------------------------------------------------|-------------------------|------------------------|
|    |                                                  | As cast                 | Beta ann. <sup>2</sup> |
| 40 | 90Ti-6Al-4V                                      | Large                   | 2                      |
|    | 90Ti-6Al-4V + .01Y                               | do                      | 1                      |
|    | 90Ti-6Al-4V + .03Y                               | Medium                  | 2                      |
|    | 90Ti-6Al-4V + .05Y                               | Small                   | 3                      |
|    | 90Ti-6Al-4V + .10Y                               | do                      | 4                      |
|    | 90Ti-6Al-4V + .15Y                               | do                      | 5                      |
|    | 90Ti-6Al-4V + .10Y <sub>2</sub> O <sub>3</sub>   | do                      | 4                      |
|    | 90Ti-6Al-4V + .20Y <sub>2</sub> O <sub>3</sub>   | do                      | 5                      |
|    | 92.5Ti-6Al-2.5Sn                                 | Large                   | 1                      |
|    | 92.5Ti-6Al-2.5Sn + .05Y                          | Small                   | 2                      |
|    | 73Ti-13V-11Cr-3Al                                | Large                   | 1                      |
|    | 73Ti-13V-11Cr-3Al + .05Y                         | Small                   | 3                      |
|    | 100Ti                                            | Large                   | 1                      |
|    | 100Ti + 1Y                                       | do                      | 1                      |
|    | 100Ti + 1Y <sub>2</sub> O <sub>3</sub>           | do                      | 1                      |
|    | 92.5Ti-5Al-2.5Sn-1Y <sub>2</sub> O <sub>3</sub>  | Small                   | 4                      |
|    | 73Ti-13V-11Cr-3Al-1Y <sub>2</sub> O <sub>3</sub> | do                      | 3                      |
|    | 97Ti-1.5Al-1V                                    | Large                   |                        |
|    | 97Ti-1.5Al-1V-1Y                                 | Medium                  |                        |
|    | 95Ti-3Al-2V                                      | Large                   |                        |
|    | 95Ti-3Al-2V-1Y                                   | Medium-small            |                        |
| 55 | 86Ti-5Al-9Sn-4Y                                  |                         | 3                      |
|    | 86Ti-5Al-9Sn-4Y                                  |                         | 5                      |

<sup>1</sup> Grain sizes.—ASTM numbers and L, M and S for large, medium and small.

<sup>2</sup> Sheet (0.040-inch) annealed 50° F. above the beta transi temperatures.

In the drawing:

FIG. 1 is a photograph of a macroetched surface of a titanium-base alloy product in which there is no yttrium; and

FIG. 2 is a photograph of a macroetched surface of a similar product similarly treated, but containing 0.15 percent by weight yttrium.

Each figure shows a macroetched surface of a popular titanium-base alloy which nominally contains 6 percent by weight aluminum, 4 percent by weight vanadium, and the balance substantially titanium ("6-4" alloy). In each instance the alloy was forged from an 8 inch diameter ingot to a billet about 4 inches in diameter, and was re-

heated as required between forging operations. The work thus performed on the alloy was sufficient to achieve a

strate that increasing amounts of yttrium lowers the tensile strength more and more.

TABLE 3.—TENSILE PROPERTIES OF COMMERCIAL Ti-6Al-4V 0.625" BAR WITH YTTRIUM ADDITIONS

| Heat number | Composition                      | UTS,<br>K.s.i. | YS,<br>K.s.i. | El,<br>percent | R.A,<br>percent |
|-------------|----------------------------------|----------------|---------------|----------------|-----------------|
| 29055       | Ti-6.4Al-4.3V-0.18Fe-0.17O       | 155            | 135           | 8.5            | 18.0            |
| 29059       | Ti-6.4Al-4.3V-0.18Fe-0.17O+0.05Y | 160            | 129           | 12.5           | 29.1            |
| 29060       | Ti-6.4Al-4.3V-0.18Fe-0.17O+0.10Y | 148            | 127           | 12.7           | 32.2            |
| 29061       | Ti-6.4Al-4.3V-0.18Fe-0.17O+0.20Y | 145            | 125           | 12.5           | 33.3            |

<sup>1</sup> 1,840 F.-1 hr.-AC.

desirable fine grain size regardless of whether the alloy contained yttrium. The alloy shown in FIG. 1 (Heat No. X29297-1) in which yttrium is absent has an objectionably spangled surface. The alloy shown in FIG. 2 (Heat No. X29299-1) has no spangled surface.

Table 2, which follows, demonstrates the effect of yttrium additions in increasing the sensitivity of sonic testing for flaws in billets of "6-4" alloy. A "No. 5 Hole Test" is a sonic test adjusted to locate flaws  $\frac{5}{32}$  inch or more in diameter internally of a test specimen. A "No. 3 Hole Test" is a similar test adjusted to locate flaws  $\frac{3}{32}$  inch or more in diameter. The results of the test are observed on an oscilloscope. The "Noise" is the percent of the oscilloscope scale reading which is induced by back scatter within the test specimen where there is no measurable flaw.

TABLE 2.—EFFECT OF YTTRIUM ADDITION ON INCREASING SONIC TESTING SENSITIVITY OF Ti-6Al-4V BILLET<sup>1</sup>

| Heat number         | Percent                       |         | Billet size,<br>inches | Number 5 hole test <sup>2</sup><br>Number 3 hole test <sup>2</sup> |                     | Number 3 hole test 2 <sup>3</sup><br>Number 3 hole test 2 <sup>3</sup> |            |
|---------------------|-------------------------------|---------|------------------------|--------------------------------------------------------------------|---------------------|------------------------------------------------------------------------|------------|
|                     | Y <sub>2</sub> O <sub>3</sub> | Yttrium |                        | Background, percent                                                | Background, percent | Ave. noise                                                             | Max. noise |
| X29297              | 0                             | 0       | 5.5, square            | 35                                                                 | 11                  | 75                                                                     | 17         |
| X29298              | 0.09                          | 0.07    | do                     | 15                                                                 | 5.5                 | 50                                                                     | 11         |
| X29299              | 0.19                          | 0.15    | do                     | 20                                                                 | 5.5                 | 55                                                                     | 11         |
| X29297-1 (Figure 1) | 0                             | 0       | 4, round               | —                                                                  | —                   | 30                                                                     | —          |
| X29298-1            | 0.09                          | 0.07    | do                     | —                                                                  | —                   | 10                                                                     | —          |
| X29299-1 (Figure 2) | 0.19                          | 0.15    | do                     | —                                                                  | —                   | None                                                                   | —          |

<sup>1</sup> Background noise due to grain structure interferes with the sensitivity of sonic testing for smaller defects.

<sup>2</sup> Tested for defect levels of  $\frac{5}{32}$  and  $\frac{3}{32}$  inch hole diameter. Noise level is percent of defect scale range.

<sup>3</sup> Background noise interferes when sonic testing at a smaller defect size.

However, we have further discovered that adding yttrium to titanium-base alloys usually has an undesirable side effect in that it lowers the tensile strength of the product. In our aforementioned earlier application, we gave test results which might lead one to the opposite conclusion, but we obtained these results with tests on sheet material which had been worked and annealed at relatively low temperatures. Hence the results were not representative of products of heavier cross section, such as bar stock. The latter products must be worked at higher temperatures that is, above or near the beta transus. If the alloy is not worked at low temperatures, our more recent tests demonstrate that addition of yttrium tends to lower both the yield strength and ultimate tensile strength of many titanium-base alloy products by as much as 10K s.i.

Table 3, which follows, shows the results of tensile tests we performed on a series of 0.625 inch bars formed of "6-4" alloy. In these tests we maintained the oxygen content at 0.17% and increased the yttrium content of the different bars from nil to 0.20%. The results demon-

tanium ("6-6-2" alloy) commonly has an oxygen content of about 0.16% by weight. When we add yttrium, we may compensate for the loss in tensile strength by raising the oxygen content again by about 0.01 to 0.06%. We may achieve similar compensation by adjusting the content of other strengthening agents, notably nitrogen, which is a more potent strengthening agent than oxygen. Both the "6-4" and the "6-6-2" alloys commonly have a nitrogen content of about 0.01% by weight. When we add yttrium to these alloys, we may compensate by raising the nitrogen content by about 0.01 to 0.03%. Our preference for using oxygen is due to the fact that we can simply add yttrium oxide to the alloy, leave everything else the same, and the oxygen present in the oxide supplies the increased content of strengthening agent.

Table 4, which follows, shows the results of tensile tests we performed on series of 0.625 inch bars formed of "6-4" alloy and "6-6-2" alloy. In these tests we tested control specimens of each alloy, specimens in which we added yttrium without adjusting the oxygen content, and other specimens in which we added yttrium and adjusted the oxygen content in accordance with the present invention.

TABLE 4.—TENSILE PROPERTIES OF COMMERCIAL Ti-6Al-4V AND Ti-6Al-6V-2Sn 0.625" BAR WITH YTTRIUM AND YTTRIUM OXIDE ADDITIONS

| Heat number | Composition                                                        | Aim oxygen, percent in— |                               | Measured oxygen percent | Heat treatment    | UTS, K.s.i. |        | YS, K.s.i. |         | El, percent | RA, percent |
|-------------|--------------------------------------------------------------------|-------------------------|-------------------------------|-------------------------|-------------------|-------------|--------|------------|---------|-------------|-------------|
|             |                                                                    | Base                    | Y <sub>2</sub> O <sub>3</sub> |                         |                   | K.s.i.      | K.s.i. | percent    | percent |             |             |
| 29220       | Ti-6.4Al-4.3V-0.18Fe                                               | .170                    | —                             | 204                     | 1,840 F.-1 hr.-AC | 157         | 131    | 8.2        | 15.5    | —           | —           |
| 29200       | Ti-6.4Al-4.3V-0.18Fe+0.1Y                                          | .170                    | —                             | 160                     | 1,840 F.-1 hr.-AC | 148         | 127    | 12.7       | 32.0    | —           | —           |
| 29243       | Ti-6.4Al-4.3V-0.18Fe+0.1Y                                          | .197                    | —                             | 196                     | 1,840 F.-1 hr.-AC | 146         | 125    | 14.0       | 33.1    | —           | —           |
| 29221       | Ti-6.4Al-4.3V-0.18Fe+0.11Y <sub>2</sub> O <sub>3</sub>             | .147                    | .023                          | 186                     | 1,840 F.-1 hr.-AC | 161         | 127    | 11.7       | 32.0    | —           | —           |
| 29224       | Ti-6.4Al-4.3V-0.18Fe+0.11Y <sub>2</sub> O <sub>3</sub>             | .170                    | .023                          | 208                     | 1,840 F.-1 hr.-AC | 155         | 132    | 11.5       | 29.7    | —           | —           |
| 29241       | Ti-6.6Al-5.6V-2.18Sn-0.7Cu-0.7Fe                                   | .160                    | —                             | 184                     | 1,800 F.-1 hr.-FC | 144         | 127    | 13.5       | 22.7    | —           | —           |
| 29245       | Ti-5.6Al-5.6V-2.18Sn-0.7Cu-0.7Fe+.09Y                              | .160                    | —                             | 182                     | 1,800 F.-1 hr.-FC | 140         | 125    | 15.0       | 27.2    | —           | —           |
| 29244       | Ti-5.6Al-5.6V-2.18Sn-0.7Cu-0.7Fe-.09Y                              | .183                    | —                             | 190                     | 1,800 F.-1 hr.-FC | 145         | 129    | 15.0       | 26.9    | —           | —           |
| 29247       | Ti-5.6Al-5.6V-2.18Sn-0.7Cu-0.7Fe+.011Y <sub>2</sub> O <sub>3</sub> | .137                    | .023                          | 175                     | 1,800 F.-1 hr.-FC | 141         | 127    | 15.5       | 27.3    | —           | —           |
| 29246       | Ti-5.6Al-5.6V-2.18Sn-0.7Cu-0.7Fe+.011Y <sub>2</sub> O <sub>3</sub> | .160                    | .023                          | 180                     | 1,800 F.-1 hr.-FC | 141         | 126    | 14.5       | 28.1    | —           | —           |

Table 5, which follows, shows the effect of yttrium oxide additions on 0.625 inch bars of a number of other titanium-base alloys.

TABLE 5.—EFFECT OF YTTRIUM OXIDE ADDITIONS TO SEVERAL TITANIUM ALLOYS

| Heat number | Composition                      | Aim oxygen, percent in— |          | Measured oxygen, percent | Heat treatment     | UTS, K s.i. | YS, K s.i. | El, percent | RA, percent |
|-------------|----------------------------------|-------------------------|----------|--------------------------|--------------------|-------------|------------|-------------|-------------|
|             |                                  | Base                    | $Y_2O_3$ |                          |                    |             |            |             |             |
| 29249       | Ti-3Al-2.5V                      | .140                    | —        | .156                     | 1,800 F.-1 hr.-AC— | 109         | 89         | 17.7        | 41.0        |
| 29248       | Ti-3Al-2.5V-0.11 $Y_2O_3$        | .140                    | .023     | .143                     | 1,800 F.-1 hr.-AC— | 107         | 89         | 18.8        | 46.7        |
| 29252       | Ti-4Al-4V                        | .150                    | —        | .173                     | 1,800 F.-1 hr.-AC— | 124         | 103        | 15.7        | 39.9        |
| 29253       | Ti-4Al-4V-0.11 $Y_2O_3$          | .150                    | .023     | .163                     | 1,800 F.-1 hr.-AC— | 125         | 106        | 16.0        | 44.9        |
| 29261       | Ti-6Al-8V                        | .150                    | —        | .149                     | 1,750 F.-1 hr.-AC— | 157         | 131        | 10.5        | 21.8        |
| 29260       | Ti-6Al-8V-0.11 $Y_2O_3$          | .150                    | .023     | .174                     | 1,750 F.-1 hr.-AC— | 153         | 128        | 12.5        | 29.6        |
| 29258       | Ti-7Al-4Mo                       | .150                    | —        | .150                     | 1,950 F.-1 hr.-FC— | 134         | 118        | 12.0        | 19.7        |
| 29257       | Ti-7Al-4Mo-0.11 $Y_2O_3$         | .150                    | .023     | .158                     | 1,950 F.-1 hr.-FC— | 138         | 123        | 16.3        | 30.2        |
| 29256       | Ti-5Al-2.5Sn-0.2Fe               | .150                    | —        | .154                     | 1,920 F.-1 hr.-AC— | 131         | 119        | 14.0        | 23.2        |
| 29254       | Ti-5Al-2.5Sn-0.2Fe-0.11 $Y_2O_3$ | .150                    | .023     | .179                     | 1,920 F.-1 hr.-AC— | 134         | 122        | 14.0        | 31.5        |
| 29250       | Ti-8Al-1Mo-1V                    | .150                    | —        | .166                     | 1,955 F.-1 hr.-AC— | 151         | 134        | 10.7        | 18.2        |
| 29251       | Ti-8Al-1Mo-1V-0.11 $Y_2O_3$      | .150                    | .023     | .169                     | 1,955 F.-1 hr.-AC— | 144         | 124        | 13.0        | 30.5        |

From the foregoing description it is seen that our invention affords a simple, reliable method first of improving the macrostructure of a wide variety of titanium-base alloy products, and second overcoming any adverse effects on the product.

We claim:

1. A method of improving the macrostructure of titanium-base alloy products which contain about 70 to 97 percent by weight titanium, the improvement being in reduction of the grain size and in the elimination of spangled surfaces on macro-etched sections, said method comprising adding to the alloy about 0.03 to 0.40 percent by weight yttrium, and compensating for the loss of tensile properties which would otherwise result from the yttrium addition by raising the content of at least one of the strengthening agents of the group consisting of oxygen and nitrogen above the normal level present in the alloy in the absence of yttrium by amounts of about 0.01 to 0.06 percent by weight of the alloy in the case of oxygen and 0.01 to 0.03 percent by weight of the alloy in the case of nitrogen.

2. A method as defined in claim 1 in which the oxygen content is raised by about 0.01 to 0.06 percent.

3. A method as defined in claim 1 in which the nitrogen content is raised by about 0.01 to 0.03 percent.

4. A method as defined in claim 1 in which yttrium is in the form of its oxide when added, and the oxygen present in said oxide supplies the increased content of strengthening agent.

5. A method as defined in claim 1 in which the alloy nominally contains 6 percent by weight aluminum, 6 percent by weight vanadium, 2 percent by weight tin and the balance substantially titanium and has a normal oxygen content of about 0.16 percent by weight and in which com-

pensation is obtained by raising the oxygen content by about 0.01 to 0.06 percent.

6. A method as defined in claim 1 in which the yttrium

is in the form of the metal when added, and the increased content of strengthening agent is added separately.

20 7. A method as defined in claim 1 in which the alloy nominally contains 6 percent by weight aluminum, 4 percent by weight vanadium and the balance substantially titanium and has a normal oxygen content of about 0.17 percent by weight and in which compensation is obtained by raising the oxygen content by about 0.01 to 0.06 percent.

25 8. A method as defined in claim 7 in which yttrium is in the form of its oxide when added, and the oxygen present in said oxide supplies the increased content of oxygen.

30 9. A product obtained by the method of claim 1.

#### References Cited

##### UNITED STATES PATENTS

|           |         |                    |            |
|-----------|---------|--------------------|------------|
| 3,028,234 | 4/1962  | Alexander et al. — | 75—175.5 X |
| 3,070,468 | 12/1962 | Grant —            | 148—20.3   |
| 3,113,991 | 12/1963 | Kleber —           | 75—175.5 X |
| 3,141,235 | 7/1964  | Lenz —             | 75—176 X   |
| 3,205,099 | 9/1965  | Vordahl —          | 148—4      |
| 3,310,398 | 3/1967  | Kneip —            | 75—175.5 X |
| 3,360,366 | 12/1967 | Bonis —            | 75—178     |

##### OTHER REFERENCES

45 Nuclear Science Abstracts, vol. 13, No. 23, December 1959, p. 2844.

Handbook of Chemistry and Physics, 46th ed., 1965—66, p. B146.

50 Journal of Nonferrous Metals, No. 1, 1959 (Russian), Sauitskiy et al., pp. 2, 5, 9 and 10.

CHARLES N. LOVELL, Primary Examiner